

## UNITED STATES PATENT OFFICE

2,060,594

## PHOTOGRAPHIC DEVELOPER

Wilhelm Schneider, Dessau, and Gustav Wilmanns, Wolfen Kreis Bitterfeld, Germany, assignors to Agfa Ansco Corporation, Binghamton, N. Y., a corporation of New York

No Drawing. Application May 11, 1935, Serial No. 20,984. In Germany May 19, 1934

7 Claims. (Cl. 95—88)

Our present invention relates to a photographic developer.

One of its objects is a photographic developer. Another object is a photographic developer which is particularly adapted for fine grain development. Further objects will be seen from the detailed specification following hereafter.

A fine-grain development of a layer of silver halide emulsion has hitherto been produced, either by using para-phenylenediamine as the developing agents, either alone or mixed with other developing agents, or by protracting the time of development with use of usual agents, for example metol, in smaller quantity and with only a small proportion of alkali, and thus influencing the size of the grain. The first-named procedure is not satisfactory owing to the deleterious action of para-phenylenediamine on the skin. In the second method the developer is only partially consumed, since already after a short use the small proportion of alkali has been consumed.

This invention relates to a process of fine-grain development in which the developing agent used is a halogen substitution product of a 2-alkylaminophenol. The compounds are obtainable, for instance, by splitting a chloro-substituted 2-methylbenzoxazole dimethylsulfate in the presence of caustic soda and saponification of the resulting acetyl product with hydrochloric acid. With a normal content of alkali and sulfite these agents develop slowly and with fine grain without the disadvantages of the older agents referred to above. The developers have the further advantage that they do not produce fog. The position of the halogen atom in the molecule or the introduction of two halogen atoms into the molecule affords a means of rendering the developer more or less gradual in its action. As specific compounds suitable for the invention may be named: 4-chloro-2-methylaminophenol, 5-chloro-2-methylaminophenol, 4: 5-dichloro-2-methylaminophenol and 5: 6-dichloro-2-methylaminophenol.

The following examples of developers illustrate the invention:

## Example 1

45 200 cc. of water  
2 grams of 4-chloro-2-methylaminophenol  
5 grams of sodium sulfite (anhydrous)  
10 grams of potassium carbonate  
0.2 gram of potassium bromide.

The time of development at 18° C. is 10-15 minutes.

## Example 2

200 cc. of water  
1 gram of 5-chloro-2-methylaminophenol  
5 grams of sodium sulfite (anhydrous)  
10 grams of potassium carbonate  
0.2 gram of potassium bromide.

The time of development at 18° C. is 15 to 30 minutes.

## Example 3

200 cc. of water  
1 gram of 4: 6-dichloro-2-methylaminophenol  
5 grams of sodium sulfite (anhydrous)  
10 grams of potassium carbonate  
0.2 gram of potassium bromide.

The time of development at 18° C. is 30 to 60 minutes.

What we claim is:

1. A photographic developer including a halogenated 2-methylaminophenol.
2. A photographic developer including a halogenated 2-methylaminophenol and an alkali.
3. A photographic developer including a mono-halogenated 2-methylamino-phenol and an alkali.
4. A photographic developer including a di-halogenated 2-methylamino-phenol and an alkali.
5. A photographic developer comprising

200 cc. of water  
2 grams of 4-chloro-2-methylaminophenol  
5 grams of sodium sulfite (anhydrous)  
10 grams of potassium carbonate  
2.0 gram of potassium bromide.

## 6. A photographic developer comprising

200 cc. of water  
1 gram of 5-chloro-2-methylaminophenol  
5 grams of sodium sulfite (anhydrous)  
10 grams of potassium carbonate  
0.2 gram of potassium bromide.

## 7. A photographic developer comprising

200 cc. of water  
1 gram of 4: 6-dichloro-2-methylaminophenol  
5 grams of sodium sulfite (anhydrous)  
10 grams of potassium carbonate  
0.2 gram of potassium bromide.

WILHELM SCHNEIDER.  
GUSTAV WILMANNS.